

# UNITED STATES PATENT OFFICE.

WILLIAM JULES SAMUEL GRAWITZ, OF NOGENT-SUR-MARNE, FRANCE.

## PROCESS OF DYEING.

SPECIFICATION forming part of Letters Patent No. 577,295, dated February 16, 1897.

Application filed January 18, 1895. Serial No. 535,347. (No specimens.) Patented in Belgium July 9, 1894, No. 110,914; in Italy January 5, 1895, LXXIV, 292; in France January 5, 1895, No. 244,121; in Hungary January 10, 1895, No. 5,580; in England February 6, 1895, No. 2,614; in Austria February 10, 1895, No. 41, and in Spain March 30, 1895, No. 16,831.

To all whom it may concern:

Be it known that I, WILLIAM JULES SAMUEL GRAWITZ, a citizen of the Republic of France, residing in Nogent-sur-Marne, in said Republic of France, have invented certain new and useful Improvements in Processes of Dyeing or Printing Fibers in Black, or Shades Approaching Thereto, (for which Letters Patent were granted to me in Great Britain, No. 2,614, dated February 6, 1895; in Belgium, No. 110,914, dated July 9, 1894; in Spain, No. 16,831, dated March 30, 1895; in France, No. 244,121, dated January 5, 1895; in Hungary, No. 5,580, dated January 10, 1895; in Austria, No. 41, dated February 10, 1895, and in Italy, No. LXXIV, 292, dated January 5, 1895,) of which the following is a specification.

This invention relates to an improved process of dyeing or printing vegetable textile fibers, silk, or wool black, or shades approaching thereto, with anilin, its homologues, or

derivatives. Fibers which are dyed by means of a salt of anilin (or of one of its homologues or derivatives) under the oxidizing action of a chlorate (the color being developed by aging, that is, by exposing to air in aging-rooms or in aging-machines after drying) are liable to become weakened.

The object of the present invention is to overcome this defect by oxidizing the sulfo-cyanate of anilin instead of the nitrate or chlorhydrate or other salts already used for the transformation in black.

The sulfo-cyanate of anilin may be obtained in combining directly the sulfo-cyanic acid ( $\text{CHNS}$ ) with the anilin. It may also be obtained by double decomposition. In mixing, for example, a solution of sulfo-cyanate of barium ( $\text{CNS}_2\text{Ba} + 2\text{H}_2\text{O}$ , with a heated solution of sulfate of anilin, a soluble sulfo-cyanate of anilin and an insoluble sulfate of barium are formed according to the following equation:



The sulfate of barium is then separated by filtering and a pure solution of sulfo-cyanate of anilin is obtained. The sulfo-cyanate of anilin is also formed by mixing the nitrate or the hydrochlorate of anilin with a soluble sulfo-cyanate, such as that of barium, calcium, or ammonia; but in these cases the sulfo-cyanate of anilin cannot be separated because the nitrates or the chlorides of barium, calcium, or ammonium, which have been formed by double decomposition, are themselves soluble like the sulfo-cyanate of anilin; but such a mixture acts practically in the same manner as the purified and isolated sulfo-cyanate of anilin. On the contrary, by mixing a solution of a salt of anilin, such as nitrate or hydrochlorate of anilin, with an insoluble sulfo-cyanate no double decomposition will take place.

I would have it understood that two or more soluble sulfo-cyanates may be used together, similarly that two or more salts of anilin may be employed together, for instance, hydrochlorate of anilin and nitrate of anilin, likewise that vanadate of ammonia may be used conjointly with another soluble vana-

date. In the same way chlorate of potash may be substituted for chlorate of soda or for any other soluble chlorate, or several may be used together, as well known. I do not confine myself to the use of pure anilin that yields black, as this process is applicable to its homologues, such as toluidins, xylidins, orderivatives, such as paraphenylenediamin, and in general to all artificial amins known to yield colors approaching black with the decomposition products of the chlorates, whether for printing or for dyeing purposes and whether the matters to be treated are unbleached or dyed, in the raw state, spun or woven, or in course of manufacture.

I will here indicate, merely by way of two examples, the preparation of the dye-baths.

First example: Anilin salt, (hydrochlorate or one equivalent,) twelve hundred and ninety-five grams; sulfo-cyanate (soluble) of ammonia, crystallized, or one equivalent, seven hundred and sixty grams; chlorate of soda, two-thirds of an equivalent containing four equivalents of oxygen, seven hundred and ten grams.

Second example: Anilin salt, (hydrochlor-

rate,) twelve hundred and ninety-five grams; sulfo-cyanate (soluble) of ammonia, crystallized, seven hundred and sixty grams; crystallized chlorid of manganese, seven hundred and fifty grams; chlorate of soda, seven hundred and ten grams.

In both examples the substances are dissolved separately and mixed lukewarm, while I add enough water to make a total volume of thirteen liters, and after cooling I add to the bath one gram of vanadate of ammonia dissolved in one hundred grams of water. The fibrous materials impregnated with this mixture take a magnificent black by aging, that is, by exposing to air in aging-rooms or aging-machines. By progressively increasing the proportion of the chlorate as much as six equivalents of oxygen may be supplied.

I would have it understood that the proportion above indicated may be varied. I can greatly diminish, for instance, the proportion of the sulfo-cyanate, as the sulfo-cyanate appears to have a specific preservative action.

In conclusion I would remark that in order to obtain a good color on silk it is preferable

to repeat the dyeing operation two or more times.

The wool chlorinated as indicated by Lightfoot or treated by any other known process can be well dyed black with my process.

Having thus described my invention, I claim as new and desire to secure by Letters Patent—

The process herein described of dyeing or printing vegetable textile fibers, prepared wool or silk by means of the sulfo-cyanate of anilin or its homologues as set forth, which consists in treating the fibers with a mixture of a salt of anilin with a soluble cyanate capable of forming the sulfo-cyanate of anilin by double decomposition, and developing the color by the oxidizing of the chlorate in presence of a salt of vanadium, substantially as described.

In testimony that I claim the foregoing as my invention I have signed my name in presence of two subscribing witnesses.

WILLIAM JULES SAMUEL GRAWITZ.

Witnesses:

GREGORY PHELAN,

EDOUARD HENRIQUEZ.